

No. 891,265.

PATENTED JUNE 23, 1908.

C. T. KNIPP.

PROCESS FOR PURIFICATION OF METALS.

APPLICATION FILED AUG. 6, 1907.



WITNESSES:

L. S. Dancy

H. A. McCrea

C. T. Knipp

INVENTOR.

By James Hamilton  
ATTORNEY.

# UNITED STATES PATENT OFFICE.

CHARLES T. KNIPP, OF URBANA, ILLINOIS.

## PROCESS FOR PURIFICATION OF METALS.

No. 891,265.

Specification of Letters Patent.

Patented June 23, 1908.

Application filed August 6, 1907. Serial No. 387,871.

*To all whom it may concern:*

Be it known that I, CHARLES T. KNIPP, a citizen of the United States, residing at Urbana, in the county of Champaign and State of Illinois, have invented certain new and useful Improvements in Processes for Purification of Metals, of which the following is a specification, reference being had to the accompanying drawings.

10 My invention relates to improvements in processes for the purification of metals; and an object of my invention is to provide a process which will result in removing practically all the impurities from the metal and which will be simple, economical and efficient.

15 The mercury still described in my pending application Serial No. 329,619 filed August 7, 1906, is one form of apparatus for carrying out my new process.

As applied to the purification of the metal, mercury, for example, my new process consists in vaporizing the metal by an electric arc and *in vacuo*; and then condensing the vapor out of contact with the impure metal and leading away the distillate.

20 The mercury is separated into two portions which in the still form the electrodes of an electric arc; the pressure upon the mercury being reduced as far as possible by exhausting the air from the still as far as possible. The heat from the electric arc volatilizes the mercury and the mercury vapor flows into another chamber of the still, 25 known as the condensing chamber, and is there condensed out of contact with the impure mercury. The distillate flows from the condensing chamber and passes through a capillary tube connected therewith, whereby 30 the vacuum in the still is maintained; but it is not to be understood that this air-pump action of the distillate is an essential step in my new process, for the vacuum may be maintained by other well-known means.

40 An apparatus for carrying out my invention is shown in the drawing, in which

Figure 1 is an elevation of the apparatus and Figs. 2 and 3 illustrate modifications hereinafter referred to.

50 The ends of the tube A are bent downwardly and formed with the bulbs B, C from each of which extends a small bore tube D, the lower end of which dips into a vessel E'. Intermediate the bulbs B, C the tube A is formed with a recess or pocket F in the bot-

tom of which is fused a platinum wire G for a purpose hereinafter referred to.

The tube A is in communication with (opens into) one end of the condensation tube H the other end of which is extended downwards by the tube I which terminates in an S provided with an enlargement or reservoir J. The upper portion I' of the tube I is of comparatively large bore, while the lower portion I'' of the tube I is of small bore, 60 or a capillary tube. Between the portions I' and I'' is an enlargement or chamber S within which is a hollow valve S', which prevents any flow of mercury from the reservoir S into the capillary tube I'' except through the valve itself. From near the top of the valve S' extends downwardly a tubular inlet arm h which reaches to near the bottom of the chamber S; and extending upwardly from the valve is a vent-piece v which permits air 65 to be exhausted from the capillary tube I'' through the valve S'. The latter traps the mercury in the bulb S; and when the mercury has reached the level of the point of junction of the arm or inlet tube h with the top of the valve S', the mercury will escape through the valve S' into the capillary tube I''. In this way any dross or impurity floating on the top of the mercury in the chamber S is prevented 70 from escaping into the capillary tube I''. 75

The condensation tube H is provided with the condensation chamber K and is formed with a nipple L for the attachment of a rubber hose or like means of connection to a Geryk hand or power air-pump (not shown), 80 or other equally effective air-pump.

85 The upper portions of the tubes D and I are made separate from their lower portions as is indicated at U, U' U''. This construction enables the upper part of the apparatus to be separated from the lower part, for the purpose of cleaning. When the apparatus is in use, the spaces U, U' U'' are bridged over or closed by a piece of rubber tubing r. When the tubing is new, it will be found generally to suffice in keeping the joints air-tight. In order to reinforce the tubing r and hermetically seal the joint, a jacket made up of a cork c and tube t filled with mercury m is used. Although only one of the joints (that marked U) is shown fitted with this ferrule, it will be understood that the other two joints U', U'' are also sealed, when the apparatus is in use.

100 The mercury in one of the vessels E' is con- 110

nected with the negative pole of a suitable source of electric current, as a dynamo, storage battery or the like. Preferably direct current is used. The mercury in the other 5 vessel E' is electrically connected through the resistance R with the positive pole of the source of electric current; and with this same positive pole the platinum wire G of the side connection F is connected through the 10 resistance R'. Of course, it will be understood that the mercury in the tubes D and the bulbs B, F and C serve as conductors for the electric current. The mercury in the bulb C acts as a return circuit for the current 15 which flows through the mercury in the bulbs B and F.

The length of the capillary portion I'' of the tube I is such that the level of the column of mercury sustained by the atmosphere in 20 the capillary tube I'' is about five centimeters below the bottom of the chamber S. The volume of the bulb J is sufficient to insure against the admission of air.

The vessels E' are made with their upper 25 portions wide and shallow or dish-shaped, and resemble somewhat a frying pan from which extends downwardly a pipe. This shape enables the vessels E' to hold a large volume of mercury without altering in a 30 great degree the mercury level in the bulbs B and C.

To start the still: Place a beaker E<sup>x</sup> of clean mercury at the lower end of the tube I'' allowing the latter to dip into it, as shown 35 by the dotted outline. Place the vessels E' in position as shown and fill with the mercury to be distilled. Connect the nipple L to an air-pump, (a Geryk hand or power pump is well adapted for this purpose), and slowly 40 exhaust the air from the still. The mercury will rise in the tubes I and D, and after 15 or 20 minutes of pumping, it will become stationary. Clearly the columns of mercury are supported by the pressure of the atmosphere. Now adjust the position of one of 45 the vessels E' until the mercury stands in the bulb B at the level indicated in the drawing. Next raise the other vessel E', until the mercury rises in the bulb C and overflows, filling 50 the pocket F, after which the vessel E' is lowered so that the column stands in the bulb C at the level indicated by the heavy shading. The volume of the bulb J is sufficient to insure against the admission of air, 55 hence, the beaker E<sup>x</sup> at the lower end of I'' may now be lowered to the position indicated by the full line sketch. Electrical connections are now made as indicated in the drawing. There is a divided circuit, one branch 60 of which includes the resistance R and the mercury in the bulb B, while the other branch includes the resistance R' and the mercury in the pocket F; the common return for the two branches is the mercury in the bulb C. 65 The side connection F is purely to start the

arc between the electrodes B and C as described by Weintraub, *Phil. Mag.*, Vol. VII, February, 1904, but the arc may be started quite readily by dispensing with the side connection F and simply raising the level of the 70 mercury columns in the bulbs B and C by raising the vessels E' until the two columns touch, and then lowering the vessels. Or it may be started by the method of using a high potential discharge, as originally used by 75 Hewitt and others.

After the arc is once started between the bulbs B and C (by the Weintraub method), the circuit through the side connection F is broken. The mercury vapor fills the tube A, 80 the tube H and the condensation bulb or chamber K, upon the walls of which it condenses. The shape and position of the tube H and the condensation chamber K are such that the condensed mercury is diverted into 85 the tube I and thence is discharged through the valve S' into the beaker E<sup>x</sup> placed to receive the distillate as shown in the full lines in the drawing. As the purified metal falls drop by drop through the capillary tube I'', 90 it operates as in an air-pump of the Sprengel type and tends to maintain the vacuum produced by the Geryk pump used in starting the apparatus. However, experience indicates that it is advisable to operate the latter 95 pump from time to time, especially if the impurities give off gases, as they are very liable to do. If desired, the tube may be made of the same bore throughout, the bore being the same as that of the upper portion I', in which 100 case the chamber S is omitted but the S-shaped end and the bulb J are retained. (See Fig. 2, in which I<sup>x</sup> is the tube). In this case the dropping of the purified mercury will not operate to maintain the vacuum. 105 Again, the discharge of the purified mercury may be made to take place through a straight tube I<sup>xx</sup>, (Fig. 3), dipping into a vessel, as do the tubes D into the vessels E'.

The theory underlying the hereinbefore 110 described process may be stated as follows: It is well known that a metal in the liquid state, *e. g.*, mercury, gives off a vapor to a greater or less extent. The amount of vapor given off depends upon the temperature and 115 upon the pressure,—being excessively small when the temperature of the liquid is little above the melting point of the metal. Let us consider the case when the pressure is kept constant—when the liquid metal is contained 120 in an open dish. The pressure is that of the atmosphere. The amount of metal vapor given off will steadily increase as the temperature is raised until the boiling point is reached when there will be a great evolution 125 of vapor. At this point, as is the case of non-metallic liquids, the temperature remains constant until all of the liquid is vaporized. The addition of more heat simply hastens the vaporization without rise in tem- 130

perature. Now consider the case when the temperature is kept constant and the pressure varied. To realize this case the liquid is placed in an inclosure connected to a pump capable of increasing or decreasing the pressure at will within the vessel. If the pressure is increased, the amount of vapor given off is lessened, while if the pressure is decreased, the vessel is exhausted, the amount of vapor given off is increased. If the exhaustion is carried to completion, nothing but metallic vapor remains in the inclosure. If now, in addition, heat is supplied to the vessel, it will be found in general that but little rise in temperature is necessary to cause a great evolution of vapor. In other words, a liquid (either metallic or non-metallic) will boil, and consequently evolve its vapor at a much reduced temperature, if the pressure is reduced. This theory is directly applicable to the process in question. The still being well exhausted of air means that the mercury vapor will be given off copiously at a much lower temperature than it would be where the mercury is boiled at atmospherical pressure. The lower the temperature under which the still operates, the less liable are the impurities, such as zinc, copper, lead, etc., that are held in solution by the mercury, to be carried over into the distillate. These impurities, and others that may be found, all have melting points considerably above the boiling point of mercury in air. If the mercury is boiled in a partial vacuum or a nearly perfect vacuum, the chances of the impurities being carried over are much less; because, as pointed out above, the amount of vapor given off by a solid metal is proportional to the temperature, which in the case assumed is comparatively low.

In the process hereinbefore described, a vacuum is necessary for two reasons, (a) to maintain the arc, and (b) because a high vacuum means a low temperature at which the mercury is vaporized. If the vacuum is not high, the temperature of the arc rises rapidly and the high temperature tends to vaporize the impurities. The temperature as registered by a copper-platinum thermocouple placed within the still at the mouth of the condensing chamber is about 160 degrees centigrade when the still is run at the normal rate. The temperature of boiling mercury in air is 360 degrees centigrade.

The action of the current flowing through the still is not only to heat and vaporize the mercury but the electric forces ionize the mercury vapor as well. The complete processes that the vapors within the still undergo are not fully understood, especially when there are vapors of various metals, (in this case considered impurities) present. That there is a suppressive action on the, say zinc, ions is evident when a comparative study of the various methods is made. It was found by tests of great refinement that the distillate produced by my new process for a given sample of mercury that was slightly impure to zinc was of much greater purity than the distillate from any of the other approved low pressure stills that have been recently described. This higher degree of purity may be ascribed to (a) the low temperature that obtains in the mercury arc still; (b) the ionization processes within the tube; and (c) the high vacuum that is necessary to maintain the arc.

This application is filed as a divisional application which claims the process described as being carried out by the apparatus claimed in my pending application hereinbefore referred to.

I claim:

1. A process for the purification of metals consisting in generating an electric arc between two portions of the metal to be purified under a pressure lower than that of the atmosphere, thereby vaporizing the metal; and condensing the vapor produced out of contact with the impure metal.

2. A process for the purification of metals consisting in generating an electric arc between two portions of the metal to be purified under a pressure lower than that of the atmosphere, thereby vaporizing the metal; condensing the vapor produced out of contact with the impure metal; and maintaining the low pressure upon the impure metal by leading the distillate away drop by drop.

In witness whereof I have hereunto set my hand in the presence of the two undersigned witnesses at said Urbana this second day of August, 1907.

CHAS. T. KNIPP

Witnesses:

LEWIS A. MCLEAN,  
L. E. GAILEY.